

## UNITED STATES PATENT OFFICE

VICTOR ENGELEHARDT, OF BERLIN-CHARLOTTENBURG, GERMANY, ASSIGNOR TO SIEMENS & HALSKE, AKTIENGESELLSCHAFT, OF SIEMENSSTADT, NEAR BERLIN, GERMANY, A CORPORATION OF GERMANY

## METHOD FOR REMOVING CHLORINE IONS FROM ELECTROLYTIC SOLUTIONS

No Drawing. Application filed December 15, 1926, Serial No. 155,106, and in Germany December 31, 1925.

This invention relates to a new and useful method for removing chlorine ions from electrolytic solutions, especially from chlorinated liquid electrolytes or lyes containing zinc or other metals.

In the electrolysis of sulphate bearing solutions, as for instance of lyes containing sulphate of zinc, it is customary to use lead anodes. During the electrolytic process a superficial layer of peroxide of lead is formed on these anodes, as is well known in connection with storage batteries. Lead anodes are not attacked even when stopping the electrolysis because lead and peroxide of lead have only very little solubility in sulphuric acid. If the electrolyte, however, contains chlorine ions a considerable corrosion of the lead anodes takes place during the electrolytic process. In such cases peroxide of lead and also chloride of lead are present in the bath, the latter compound being highly soluble and producing therefore a very injurious effect on the anodes.

The lead ions in the electrolyte disturb the deposition of other metals, zinc etc, and the rapid disintegration of the lead of the anodes makes it practically impossible to carry out the electrolysis of such solutions with success. According to publications if an amount of chlorine ions of about 200 milligrams per litre, for instance, is present in the electrolyte a corrosion of the anodes takes place corresponding to 10-15% of the deposited zinc.

In the recovery of copper by electrolysis there are similar difficulties. Therefore it is necessary to remove the chlorine as completely as possible from the solution to be electrolyzed. It has already been proposed to add a silver salt especially sulphate of silver, to the electrolyte, in order to eliminate the chlorine by precipitating chloride of silver without introducing disturbing positive ions in the solution. But this method involves the disadvantage that colloidal chloride of silver is deposited which cannot be filtered at all, or only with great difficulty.

The present invention enables me to avoid this disadvantage. According to the invention a suitable body of silver, a plate for in-

stance, is used as an anode and the electrolyte is forced to pass through the anode chamber which is separated from the cathode chamber by a porous diaphragm. Preferably the intensity of current or the time of electrolysis is regulated in such a manner that a quantity of silver equivalent to the amount of chlorine is introduced in the solution. Since the operation is conducted at ordinary temperature (without heating), this quantity of silver will at once precipitate the chlorine as flaky silver chloride which is insoluble in the electrolyte at such temperature and in this state is easily filtered. The cathode chamber is charged with electrolyte free of chlorine. It will be understood that the voltage employed must be sufficient to produce the result stated, that is, to cause the silver to be dissolved.

If desired I may use intensities of electric current higher than the value above mentioned or to use a longer time for electrolysis. In such cases the excess of silver in the solution must be eliminated afterwards in order to avoid losses of silver and to obtain a pure cathode deposit when electrolyzing the lye free of chlorine. The removal of the excess of silver may be effected by the well known cementation process or electrolytically, as has been proved by experiments. After passing through the anode chamber in the manner set forth and after subsequent filtering the silver-containing lye is brought into the cathode chamber. Because of its favourable potential of deposition the silver is quantitatively precipitated on the cathode and can be recovered.

This method affords the advantage that the amount of chlorine in the solution to be electrolyzed need not be determined continuously for regulating the current intensity accordingly. Instead of pure silver, silver alloys may be employed for carrying this invention into effect, and I desire it to be understood that where the appended claims refer to silver anodes, anodes made of silver alloys are covered as equivalents.

What I claim as my invention and desire to be secured by Letters Patent is:

The method of removing chlorine ions from

metal-bearing chlorinated liquid electrolytes,  
which consists in electrolyzing the liquid with  
a silver anode at a voltage sufficient to dis-  
solve silver, for a length of time sufficient to  
cause a quantity of silver ions at least chem-  
ically equivalent to the quantity of chlorine  
ions present to be dissolved in the electrolyte,  
at a temperature at which silver chloride is  
insoluble in such electrolyte, with a resulting  
10 precipitation of silver chloride in a flaky con-  
dition.

In testimony whereof I affix my signature.  
VICTOR ENGELHARDT.